



US006753543B2

(12) **United States Patent**  
Yanagita et al.

(10) Patent No.: US 6,753,543 B2  
(45) Date of Patent: Jun. 22, 2004

(54) RADIATION IMAGE CONVERSION PANEL

(75) Inventors: **Takafumi Yanagita**, Tokyo (JP);  
**Nobuhiko Takashima**, Tokyo (JP)

(73) Assignee: **Konica Corporation**, Tokyo (JP)

(\*) Notice: Subject to any disclaimer, the term of this patent is extended or adjusted under 35 U.S.C. 154(b) by 77 days.

(21) Appl. No.: 10/098,668

(22) Filed: Mar. 15, 2002

(65) **Prior Publication Data**

US 2002/0195578 A1 Dec. 26, 2002

(30) **Foreign Application Priority Data**

Apr. 2, 2001 (JP) ..... 2001-103095  
May 24, 2001 (JP) ..... 2001-155182

(51) Int. Cl.<sup>7</sup> ..... C09K 11/61  
(52) U.S. Cl. ..... 250/581; 250/582  
(58) Field of Search ..... 250/581, 582,  
250/483.1, 483.2, 484.3, 484.4; 430/139

(56) **References Cited**

## U.S. PATENT DOCUMENTS

4,962,578 A \* 10/1990 Saito et al. .... 492/53

|           |    |   |        |                  |       |           |   |
|-----------|----|---|--------|------------------|-------|-----------|---|
| 5,237,915 | A  | * | 8/1993 | Rounslay         | ..... | 100/162   | R |
| 5,877,504 | A  | * | 3/1999 | Yanagita et al.  | ..... | 250/484.4 |   |
| 5,888,647 | A  | * | 3/1999 | Yamane           | ..... | 428/338   |   |
| 5,952,666 | A  | * | 9/1999 | Nakano et al.    | ..... | 250/484.4 |   |
| 6,262,424 | B1 | * | 7/2001 | Yanagita et al.  | ..... | 250/483.1 |   |
| 6,531,073 | B1 | * | 3/2003 | Wakamatsu et al. | ..    | 252/301.4 | H |

\* cited by examiner

*Primary Examiner*—Constantine Hannaher

Assistant Examiner—Otilia Gabor

(74) *Attorney, Agent, or Firm*—Frishauf, Holtz, Goodman & Chick, P.C.

(57) ABSTRACT

A method for preparing a radiation image conversion panel, which comprises the steps of:

- (a) applying onto a support a stimulable phosphor coating composition comprising a stimulable phosphor and a polymer resin to form a stimulable phosphor layer;
  - (b) drying the stimulable phosphor layer; and
  - (c) subjecting the stimulable phosphor layer on the support to a compression treatment employing a calender roller which comes into contact with the stimulable phosphor layer to form the radiation image conversion panel, wherein the calender roller comprises a resin and the surface of the calendar roller has a Shore D hardness of D80 to D97°.

**9 Claims, 1 Drawing Sheet**



FIG. 1



FIG. 2



## RADIATION IMAGE CONVERSION PANEL

## FIELD OF THE INVENTION

The present invention relates to a radiation image conversion panel employing stimulable phosphors, and an image formation method using the panel. Specifically the present invention relates to a radiation image conversion panel which results in excellent balance between the emission luminance and the sharpness of said stimulable phosphors.

## BACKGROUND OF THE INVENTION

Radiation images such as X-ray images are widely employed for medical diagnoses. Utilized as a method for obtaining X-ray images is so-called radiography in which X-rays, which have passed through an object, are subjected to irradiation onto a phosphor layer (being a fluorescent screen) to result in visible light, which is irradiated onto a silver salt bearing film, in the same manner as conventional photography, and the resulting film is subjected to photographic processing.

In recent years, however, a method has been invented in which images are formed directly from a phosphor layer instead of an image formation method employing a silver salts photographic film.

This method comprises the steps of (1) making absorbing the radiation energy which passes through the object to the phosphor; and (2) stimulating the phosphor with light or heat so that radiation energy stored in said stimulable phosphor layer is released as stimulated luminescence. (3) forming images after detecting the released energy.

Said method is described, for example, in U.S. Pat. No. 3,859,527 and Japanese Patent Publication Open to Public Inspection No. 55-12144. A radiation image conversion panel comprised of stimulable phosphors is disclosed in them.

This method uses a radiation image conversion panel and the stimulable phosphor layer of said radiation image conversion panel is subjected to radiation exposure which passes through the object being diagnosed so that radiation energy is stored corresponding to the radiation transmittance of each portion of said object. Subsequently, the resulting stimulable phosphor layer is sequentially subjected to stimulation employing electromagnetic waves (stimulating light), such as visible light and infrared rays, so that radiation energy stored in said stimulable phosphor layer is released as stimulated luminescence. Signals of the intensity variation of said stimulated luminescence are subjected, for example, to photoelectric conversion to obtain electrical signals. The resulting electrical signals are employed to reproduce visible images on recording materials such as light-sensitive films or display devices such as a CRT.

The above-mentioned image reproducing method has an advantage of using much less amount of radiation exposure compared with the conventional radiography using a combination of an intensifying screen and a conventional radiographic film. It is possible to obtain radiation images with ample information.

The stimulable phosphors employed in said radiation image conversion panel are those which result in stimulated luminescence after having been subjected to irradiation of stimulating light after said radiation. In practice, phosphors are commonly employed which result in stimulated luminescence in the wavelength range of 300 to 500 nm utilizing stimulating light in the wavelength region of 400 to 900 nm.

The radiation image conversion panel, employing said stimulable phosphors, stores radiation image information and releases stored energy through stimulating light scanning. Therefore, after scanning, it is possible to repeatedly store radiation images so as to be used repeatedly. Further, contrary to the fact that in the conventional radiography, radiographic film is consumed for every exposure, said radiation image conversion method is more advantageous from the viewpoint of resource conservation as well as economic efficiency, because it is possible to repeatedly utilize said radiation image conversion panel.

Relative advantages of radiation image conversion systems employing a radiation image conversion panel vary to large extent depending on the luminance (occasionally called sensitivity) of stimulated luminescence, as well as the image quality represented by the resultant graininess and sharpness, and these characteristics vary widely depending on characteristics of used stimulable phosphors and the configuration of the stimulable phosphor layer. In more detail, the luminescence intensity of the radiation image conversion panel, the sharpness of images, and the granularity vary depending on the size of phosphor particles, the dispersibility of said phosphors, the uniformity of phosphors, and the phosphor filling ratio. Among those, the phosphor filling ratio results in pronounced effects.

As a means to enhance said filling ratio, Japanese Patent Publication Open to Public Inspection No. 3-21893 discloses a radiation image conversion panel having a stimulable phosphor filling ratio of at least 70 percent, while employing a resin having a glass transition temperature (hereinafter occasionally referred to as Tg) of 30 to 150° C., and as an achieving means, discloses the compression of a phosphor layer (hereinafter referred simply to as a coating). The radiation image conversion panel, when employed, is slid with films as well as rollers. As a result, it is assumed that the Tg of employed binder resins is preferably at least 30° C. However, when resins having a relatively high Tg are employed as a binder resin, it becomes difficult to increase said filling ratio due to the fact that the resulting coating is not easily deformed. Further, when the finished coating is compressed, phosphors are subjected to loading due to poor softening properties of said resin, whereby light emission is degraded due to the destruction of the crystal structure of the luminous body. Further, in order to soften said resins, it is necessary to increase the compression temperature. As a result, problems have occurred in which manufacturability is degraded.

Further, Japanese Patent Publication Open to Public Inspection No. 4-44719 discloses a method to enhance the filling ratio of a phosphor layer utilizing a compression treatment. However, said patent publication does not describe any material in regard to the roller employed for said compression treatment. When simply passed between heating rollers, it was found that compression was insufficient and the phosphor was damaged. Further, said patent publication presents no suggestion in regard to the shape of the roller used. On the other hand, it was found that in the compression treatment employing a linear-shaped calender roller, said calender roller tended to warp resulting in unevenness of the compression ratio of the phosphor layer. Said unevenness induces an unevenness of the thickness of the phosphor layer, which results in sharpness fluctuation as well as granulated unevenness of the radiation image conversion panel. As a result, prompt improvement has been demanded.

In the aforesaid patent, the condition is that the temperature during heat compression is more than or equal to the Tg

of a resin. For example, the condition such as 80° C., 100° C., or the like, is described. The temperature more than or equal to the Tg of said resin, as described herein, is 69° C., which is the Tg of polyethylene terephthalate film employed widely as a support, or more than that. When a compression treatment is carried out at a temperature more than or equal to the Tg of such a support, problems occur in which said support is deformed and finally the stimulable phosphor plate is also deformed. Particularly, the deformed plate results in unevenness of luminance and sharpness during reading of images, and further results in critical problems with diagnosis. As a result, rapid improvement of these problems has been demanded.

From the view of the foregoing, the present invention has been achieved. An object of the present invention is to provide a radiation image conversion panel which exhibit an excellent balance of luminance and sharpness, and in addition, minimal sharpness fluctuation, a production method thereof, and a radiation image capturing method using the same.

#### SUMMARY OF THE INVENTION

Said object of the present invention was achieved employing the embodiments described below.

(1) A method for preparing a radiation image conversion panel, which comprises the steps of:

- (a) applying onto a support a stimulable phosphor coating composition comprising a stimulable phosphor and a polymer resin to form a stimulable phosphor layer;
- (b) drying the stimulable phosphor layer; and
- (c) subjecting the stimulable phosphor layer on the support to a compression treatment employing a calender roller which comes into contact with the stimulable phosphor layer to form the radiation image conversion panel, wherein the calender roller comprises a resin and the surface of the calender roller has a Shore D hardness of D80 to D97°.

(2) A method for preparing a radiation image conversion panel, which comprises the steps of:

- (a) applying onto a support a stimulable phosphor coating composition comprising a stimulable phosphor and a polymer resin to form a stimulable phosphor layer;
- (b) drying the stimulable phosphor layer; and
- (c) subjecting the stimulable phosphor layer on the support to a compression treatment employing a calender roller which comes into contact with the stimulable phosphor layer to form the radiation image conversion panel, wherein the calender roller has a crown value of 10 to 1,000  $\mu\text{m}$ .

(3) A method for preparing a radiation image conversion panel, which comprises the steps of:

- (a) applying onto a support a stimulable phosphor coating composition comprising a stimulable phosphor and a polymer resin to form a stimulable phosphor layer, wherein the polymer resin comprises a polymer having a glass transition point of not more than 5° C. and not less than -30° C. and the polymer accounts for at least 50 weight % of the polymer resin in the stimulable phosphor layer;
- (b) drying the stimulable phosphor layer; and
- (c) subjecting the stimulable phosphor layer on the support to a compression treatment employing a calender roller which comes into contact with the stimulable phosphor layer to form the radiation image conversion panel, wherein the temperature of the calender roller is

not less than the glass transition temperature of the polymer resin and not more than a glass transition temperature of the support.

(4) The method for preparing a radiation image conversion panel of item 1, wherein the polymer resin in the step (a) comprises a polymer having a glass transition point of not more than 5° C. and not less than -30° C. and the polymer accounts for at least 50 weight % of the polymer resin in the stimulable phosphor layer; and the temperature of the calender roller in the step (c) is not less than the glass transition point of the polymer resin and not more than a glass transition point of the support.

(5) The method for preparing a radiation image conversion panel of item 2, wherein the polymer resin in the step (a) comprises a polymer having a glass transition point of not more than 5° C. and not less than -30° C. and the polymer accounts for at least 50 weight % of the polymer resin in the stimulable phosphor layer; and the temperature of the calender roller in the step (c) is not less than the glass transition point of the polymer resin and not more than a glass transition point of the support.

(6) The method for preparing a radiation image conversion panel of item 1, wherein the compression treatment in the step (c) is carried out at a pressure of 500 to 5,000 N/cm and at a temperature of 50 to 150° C.

(7) The method for preparing a radiation image conversion panel of item 2, wherein the compression treatment in the step (c) is carried out at a pressure of 500 to 5,000 N/cm and at a temperature of 50 to 150° C.

(8) The method for preparing a radiation image conversion panel of item 3, wherein the compression treatment in the step (c) is carried out at a pressure of 500 to 5,000 N/cm.

(9) The method for preparing a radiation image conversion panel of item 1, wherein the calender roller in the step (c) has a center-line mean surface roughness Ra of 0.05 to 3  $\mu\text{m}$ .

(10) The method for preparing a radiation image conversion panel of item 2, wherein the calender roller in the step (c) has a center-line mean surface roughness Ra of 0.05 to 3  $\mu\text{m}$ .

(11) The method for preparing a radiation image conversion panel of item 3, wherein the calender roller in the step (c) has a center-line mean surface roughness Ra of 0.05 to 3  $\mu\text{m}$ .

(12) The radiation image conversion panel prepared according to the method of item 1.

(13) The radiation image conversion panel prepared according to the method of item 2.

(14) The radiation image conversion panel prepared according to the method of item 3.

(15) The radiation image conversion panel of item 12, wherein the stimulable phosphor incorporated in the stimulable phosphor layer is an Eu added BaFI compound.

(16) The radiation image conversion panel of item 13, wherein the stimulable phosphor incorporated in the stimulable phosphor layer is an Eu added BaFI compound.

(17) The radiation image conversion panel of item 14, wherein the stimulable phosphor incorporated in the stimulable phosphor layer is an Eu added BaFI compound.

(18) A method for capturing a radiation image, which comprises the steps of:

- (a) irradiating the radiation image conversion panel of item 12 from the support side of the radiation image conversion panel with X-ray which passes through an object being diagnosed so that to store a radiation energy;
- (b) stimulating the stimulable layer with an electromagnetic wave to produce stimulated luminescence; and

## 5

(c) reading the stimulated luminescence from the stimulable phosphor layer side.

(19) A method for capturing a radiation image, which comprises the steps of:

- (a) irradiating the radiation image conversion panel of item 13 from the support side of the radiation image conversion panel with X-ray which passes through an object being diagnosed so that to store a radiation energy;
- (b) stimulating the stimulable layer with an electromagnetic wave to produce stimulated luminescence; and
- (c) reading the stimulated luminescence from the stimulable phosphor layer side.

(20) A method for capturing a radiation image, which comprises the steps of:

- (a) irradiating the radiation image conversion panel of item 14 from the support side of the radiation image conversion panel with X-ray which passes through an object being diagnosed so that to store a radiation energy;
- (b) stimulating the stimulable layer with an electromagnetic wave to produce stimulated luminescence; and
- (c) reading the stimulated luminescence from the stimulable phosphor layer side.

## BRIEF DESCRIPTION OF THE DRAWINGS

FIG. 1 is a schematic view showing one example of the embodiment of the compression treatment according to the present invention; and

FIG. 2 is a schematic view showing one example of the radiation image conversion method employing the radiation image conversion panel according to the present invention.

## DETAILED DESCRIPTION OF THE INVENTION

The present invention will now be detailed.

The item (1) of the present invention is characterized in that a phosphor sheet, which has been coated with a stimulable phosphor layer (hereinafter occasionally referred simply to as a phosphor layer) and dried, is subjected to a compression treatment employing calender rollers; and said calender rollers, which come into contact with said stimulable phosphor layer, is comprised of a resin, and the Shore D hardness of its surface is from 80 to 97 degrees. Said calender rollers are preferably composed of polyester.

The compression treatment of the phosphor sheet, as described in the present invention, refers to the treatment described below. A stimulable phosphor layer is applied onto a subbed or non-subbed support and subsequently dried at desired conditions to form a stimulable phosphor layer, whereby a phosphor sheet is prepared. Subsequently, the resultant phosphor sheet is treated, for example, under the application of heat and pressure between a highly smoothed 1 to 100 cm diameter nip roller and a roller, which can be heated, facing said nip roller. By applying the compression treatment as above to said phosphor sheet, the stimulable phosphor filling ratio in said stimulable phosphor layer can be enhanced so that the luminance of emitted light can be increased, as well as enhancing the sharpness. In addition, by suitably selecting the calender roller materials, described below, the crown length, the pressure and temperature conditions, it is possible to achieve high uniformity of the phosphor sheet during compression treatment.

Compression methods employing said calender rollers are not particularly limited. It may be possible to employ any of

## 6

the methods described in "Jushi Kakoh-gijutsu Handbook (Handbook of Resin Processing Technology (edited by Kohbunshi Gakkai, Polymer Society)", edited by Nikkan Kogyo Shinbun Co., published on Jun. 12, 1965.

FIG. 1 shows one example of the embodiments of the compression treatment according to the present invention.

In FIG. 1, a stimulable phosphor layer coating composition is applied onto support 7, fed out in the conveyance direction from supply roller 6, employing coater 4. Thereafter the resulting coating is conveyed into drying zone 8 and dried employing a heated airflow from nozzles arranged on the upper and lower sides of said coating. Subsequently, support 7 (hereinafter occasionally referred to as a phosphor sheet), which has been coated with said stimulable phosphor layer and dried, is subjected to a compression treatment employing a combination of calender rollers 9-1 through 9-3, and is wound onto winding roller 10. Calender rollers are preferably comprised of calender roller 9-1, compliant roller 9-2 composed of resin, and heating roller 9-3.

In the invention according to item (1), one of the features is that the surface of the calender roller, which comes into contact with said phosphor layer, is comprised of resin of a Shore D hardness of D80 to D97 degrees and more preferably from D90 to D95 degrees.

Shore D hardness can be measured with JIS spring hardness tester (Durometer) Type D. The measuring method is described in ISO 868, ISO 7619 and JIS K7215.

The structures and types of resin of said calender roller are not particularly limited. Listed as an example may be a roller having such a configuration such that the circumferential surface of a highly rigid iron base body as an interior core is covered with, for example, an exterior cylinder made of a hard resin. Specifically listed may be Eraglass (manufactured by Kinyo Kinzoku Co.) and Mirortex Roll (manufactured by Yamanouchi Gomu Co.).

The structures and types of resin of said calender roller are not particularly limited, as long as its surface is covered with a resin having a Shore D hardness of D80 to D97 degrees. Listed as an example may be a roller having such a configuration that the circumferential surface of a highly rigid iron base body as an interior core is covered with, for example, an exterior cylinder made of hard resin. Specifically, listed may be Eraglass (manufactured by Kinyo Kinzoku Co.) and Mirortex Roll (manufactured by Yamanouchi Gomu Co.).

The Shore D Hardness (HS) of resin materials in the present invention can be measured employing commercially available apparatus. One of examples of such apparatus is a rubber-plastic hardness tester Asker Type D (manufactured by Kohbunshi Keiki Co., Ltd.).

The invention according to item (2) is characterized in that the crown value (or length) of the central portion of the calender roller with respect to both ends of said roller which comes into contact with the stimulable phosphor layer is from 10 to 1,000  $\mu\text{m}$ . Said crown length is preferably from 50 to 300  $\mu\text{m}$ . The crown value (or length), as described in the present invention, refers to an increase in height of the central portion of the roller, and specifically refers to the diameter difference (in  $\mu\text{m}$ ) between the central portion and the end of the roller. In the present invention, by specifying the crown length of the roller used to said range, the linear pressure along the full roller width can be kept constant so that uniformity during the compression treatment can be realized.

One of the embodiments of the present invention is characterized in that a compression treatment by a calender

roller is carried at a pressure of 500 to 5,000 N/cm (50 to 500 kg/cm) and a temperature of 50 to 150° C. Said pressure is preferably from 1 to 4 kN/cm, while said temperature is preferably from 50 to 100° C. By carrying out said compression treatment under conditions specified as above, the compression ratio of the stimulable phosphor layer is enhanced. As a result, the stimulable phosphor filling ratio is enhanced and high luminance, as well as excellent sharpness and graininess, can be achieved. Specifically, under said conditions, the compression ratio of the phosphor layer near the support is enhanced. As a result, effects are particularly exhibited in a method in which X-rays are irradiated onto the stimulable phosphor layer through the support of the radiation image conversion panel.

In said conditions, a sufficient compression ratio is not obtained at a linear pressure of less than 500 N/cm as well as at a temperature of less than 50° C. Further, conditions of a linear pressure of at least 5 kN/cm as well as a temperature of at least 150° C. are not preferred, since a decrease in luminance may result due to damage to stimulable phosphor particles.

One of the embodiments of the present invention is characterized in that center-line mean surface roughness Ra of a calender roller is from 0.05 to 3  $\mu\text{m}$ . Said surface roughness Ra is preferably from 0.2 to 2  $\mu\text{m}$ .

The center-line mean surface roughness Ra, as described in the present invention, is defined based on JIS B 0601 Surface roughness. Namely, the center-line mean roughness Ra, as described herein, means the value, in micrometer ( $\mu\text{m}$ ), obtained by the formula shown below, when a part of measured length L is sampled from the roughness curve in the direction of the center-line; at a cut-off value of 0.8 mm, the center-line of the sampled part is taken as the X-axis and the direction of longitudinal magnification is taken as the Y-axis; and the roughness curve is expressed by  $Y=f(X)$ .

$$Ra = \frac{1}{L} \int_0^L |f(x)| dx$$

Listed as usable measurement apparatus may be, for example, RSTPLUS non-contact 3-dimensional minute surface shape measurement system, manufactured by Wyko Co.

In the present invention, a high filling ratio can be obtained by applying the compression treatment to said phosphor sheet employing any of the methods described above. In the present invention, the filling ratio of the total stimulable phosphors in the stimulable phosphor layer is preferably at least 55 percent. Since the upper limit is naturally limited, said ratio is more preferably from 56 to 75 percent.

In the present invention, the stimulable phosphor filling ratio in the stimulable phosphor layer can be determined as described below. The radiation image conversion panel or the protective layer of the phosphor sheet is removed, and subsequently all the stimulable phosphor layer is peeled off or is dissolved out employing organic solvents. The resultant product is collected by filtration and dried. Thereafter, in order to remove the resins on the surface, the collected product is burned at 600° C. for one hour, employing an electric furnace. Said filling ratio is then obtained based on the formula described below:

$$\text{Phosphor filling ratio} = \frac{M}{(P \times Q \times R)} \times 100 \text{ (in percent)}$$

wherein M (in g) is the weight of stimulable phosphors after burning, P (in cm) is the thickness of the phosphor layer

before dissolving out, Q (in  $\text{cm}^2$ ) is the area of the phosphor sheet employed for dissolving out, and R (in  $\text{g}/\text{cm}^2$ ) is the specific gravity of the phosphor prior to dissolving out.

The present invention makes it possible to prepare a radiation image conversion panel which exhibited excellent smoothness as well as minimal image unevenness, utilizing the following. A polymer resin, having a glass transition point in the specified range, was used to prepare a stimulable phosphor layer. A phosphor sheet, which comprised a support having thereon said stimulable phosphor layer, was subjected to a compression treatment at optimal conditions such as at least Tg of said polymer resin to at most Tg of said support, which was suitable for the aforementioned characteristics.

The present invention will now be detailed.

One feature of the invention according to item 3 is characterized in that a stimulable phosphor layer comprises a polymer resin, having a glass transition point (Tg) of -30 to 5° C., in an amount of more than or equal to 50 percent by weight of the total polymer resin in said stimulable phosphor layer. The content ratio of said polymer resin is preferably from 60 to 100 percent by weight, and is more preferably from 80 to 100 percent by weight.

The glass transition point (Tg), as described in the present invention, refers to the value obtained employing the method described in Brandrup, et al., "Polymer Handbook" pages III-139 to III-179 (Wiley and Sons Co., 1966).

When a binder is comprised of a copolymer resin, the Tg is obtained based on the following formula:

$$Tg \text{ (of copolymer) (in } ^\circ\text{C.}) = v_1 Tg_1 + v_2 Tg_2 + \dots + v_n Tg_n$$

wherein  $v_1, v_2, v_3, \dots, v_n$  each represents the mass fraction of the monomer in the copolymer, and  $Tg_1, Tg_2, Tg_3, \dots, Tg_n$  each represents the Tg of the homopolymer prepared employing each monomer in the copolymer. The accuracy of the Tg calculated by said formula is  $\pm 5^\circ\text{C}$ .

Polymer resins, which are usable binders in the present invention, are not particularly limited, and include, for example, polyurethanes, polyesters, vinyl chloride copolymers, vinyl chloride-vinyl acetate copolymers, vinyl chloride-vinylidene chloride copolymers, vinyl chloride-acrylonitrile copolymers, butadiene-acrylonitrile copolymers, polyamide resins, polyvinyl butyral, cellulose derivatives (nitrocellulose), styrene-butadiene copolymers, various types of synthetic rubber, phenol resins, epoxy resins, urea resins, melamine resins, phenoxy resins, silicone resins, acryl based resins, and urea-formamide resins. Of these, polyurethanes, polyesters, and vinyl chloride based copolymers are preferably employed.

The present invention is characterized in comprising a polymer resin having a glass transition point (Tg) of -30 to 5° C. in an amount of at least 50 percent by weight based on the total polymer resins of the stimulable phosphor layer. Other polymer resins, known in the art, may be employed which exhibit characteristics other than those specified above.

In the present invention, polymer resins comprised of resins, having a hydrophilic polar group, are more preferably employed. It is assumed that the adsorption of said hydrophilic polar group onto the surface of stimulable phosphor particles improves the dispersibility of said stimulable phosphors and also minimizes the coagulation thereof, and as a result, enhances coating stability, sharpness, and graininess. Specifically, polymer resins preferably comprise at least one of the hydrophilic polar groups selected from groups consisting of  $-\text{SO}_3\text{M}$ ,  $-\text{OSO}_3\text{M}$ ,  $-\text{COOM}$ ,  $-\text{PO}(\text{OM})_2$ , and  $-\text{OPO}(\text{OM})_2$ . M represent H or an alkali metal atom such as Li, K and Na.

Polyurethane preferably employed in the present invention will now be described, which is one example of resins having a hydrophilic polar group. Polyurethanes can be synthesized employing a commonly used method, such as utilizing a reaction between polyols and polyisocyanates. Generally employed as polyol components are polyester polyols prepared utilizing a reaction between polyols and polybasic acids. By utilizing said method, polyester polyols having hydrophilic polar groups can be synthesized employing said hydrophilic polar groups as one portion of the polybasic acid.

Further, in addition to these, polyurethane UR8300 having a  $-\text{SO}_3\text{Na}$  group (manufactured by Toyo Boseki Co.) and polyurethane TIM-6001 having a  $\text{COOH}$  group (manufactured by Sanyo Kasei Co.) are readily available as commercial products.

Further, vinyl chloride based resins, which are preferably employed, can be synthesized utilizing an addition reaction between copolymers having an OH group such as vinyl chloride-polyvinyl alcohol copolymers and compounds having the same hydrophilic polar group as described above and a chlorine atom.

Listed as commercially available these products are, for example, MR110 (manufactured by Nippon Zeon Co.) which is a vinyl chloride-vinyl acetate copolymer having a  $-\text{SO}_3\text{K}$  group. Listed as polyesters having a  $-\text{SO}_3\text{Na}$  group is Biron 330 (manufactured by Toyo Boseki Co.), and listed as polyurethane is UR-8200 having a  $-\text{SO}_3\text{Na}$  group (manufactured by Toyo Boseki Co.).

Another feature of the invention according to claim 1 is that a phosphor sheet, which is prepared by applying a stimulable phosphor layer onto a support and which is subsequently dried, is subjected to a compression treatment in the temperature range of at least the  $T_g$  of the polymer resin to at most the  $T_g$  of said support, employing calender rollers.

The compression treatment of the phosphor sheet, as described in the present invention, refers to the treatment described below. A stimulable phosphor layer is applied onto a subbed or non-subbed support and subsequently dried at desired conditions to form a stimulable phosphor layer, whereby a phosphor sheet is prepared. Subsequently, the resultant phosphor sheet is treated, for example, under the application of heat and pressure between a highly smoothed 1 to 100  $\text{cm}^2$  nip roller and a roller, which can be heated, facing said nip roller. The first effect of the application of said compression treatment applied to said phosphor sheet is that the stimulable phosphor filling ratio in said stimulable phosphor layer can be enhanced so as to increase the luminance of emitted light as well as to improve sharpness, and the second effect is that by specifying the application conditions of pressure and heat, it is possible to obtain the high uniformity of said phosphor sheet during said compression treatment.

In the followings are described about the components of radiation image conversion panels employing stimulable phosphors the present invention. Employed as stimulable phosphors for the radiation image conversion panel are, for example, phosphors which result in stimulated luminescence in the wavelength range of 300 to 500 nm, utilizing stimulating light in the wavelength region of 400 to 900 nm.

Examples of phosphors preferably used for radiation image conversion panels of the present invention are described below. However, the present invention is not limited to these examples.

(1) Rare earth element activated alkaline earth metal fluorinated halogen phosphors represented by the composi-

tion formula of  $(\text{Ba}_{1-x}, \text{M}^{II+}_x)\text{FX}_y\text{A}$ , described in Japanese Patent Publication Open to Public Inspection No. 55-12145, wherein  $\text{M}^{II+}$  represents at least one of Mg, Ca, Sr, Zn, and Cd; X represents at least one of Cl, Br, and I; A represents at least one of Eu, Tb, Ce, Tm, Dy, Pr, Ho, Nd, Yb, and Er; "x" and "y" each represent figures satisfying the relationship of  $0 \leq x \leq 0.6$  and  $0 \leq y \leq 0.2$ , respectively. Further, said phosphors may comprise additives as described in (a) through (j) below.

- (a)  $\text{X}', \text{BeX}''$ ,  $\text{M}^{III}\text{X}_3'''$ , described in Japanese Patent Publication Open to Public Inspection No. 56-74175, (wherein  $\text{X}'$ ,  $\text{X}''$  and  $\text{X}'''$  each represent at least one of Cl, Br and I; and  $\text{M}^{III}$  represents a trivalent metal);
- (b) metal oxides described in Japanese Patent Publication Open to Public Inspection No. 55-160078, such as  $\text{BeO}$ ,  $\text{BgO}$ ,  $\text{CaO}$ ,  $\text{SrO}$ ,  $\text{BaO}$ ,  $\text{ZnO}$ ,  $\text{Al}_2\text{O}_3$ ,  $\text{Y}_2\text{O}_3$ ,  $\text{La}_2\text{O}_3$ ,  $\text{In}_2\text{O}_3$ ,  $\text{SiO}_2$ ,  $\text{TiO}_2$ ,  $\text{ZrO}_2$ ,  $\text{GeO}_2$ ,  $\text{SnO}_2$ ,  $\text{Nb}_2\text{O}_5$ , and  $\text{ThO}_2$ ;
- (c) Zr and Sc described in Japanese Patent Publication Open to Public Inspection No. 56-116777;
- (d) B described in Japanese Patent Publication Open to Public Inspection No. 57-23673;
- (e) As and Si described in Japanese Patent Publication Open to Public Inspection No. 57-23675;
- (f) M-L (wherein M represents at least one alkali metal selected from the group of Li, Na, K, Rb, and Cs; L represents at least one trivalent metal selected from the group of Sc, Y, La, Ce, Pr, Nd, Pm, Sm, Gd, Tb, Dy, Ho, Er, Tm, Yb, Lu, Al, Ga, In, and Tl) described in Japanese Patent Publication Open to Public Inspection No. 58-206678;
- (g) calcined tetrafluoroboric acid compounds described in Japanese Patent Publication Open to Public Inspection No. 59-27980; calcined, univalent or divalent metal salt of hexafluorosilic acid, hexafluorotitanic acid or hexafluorozirconic acid, described in Japanese Patent Publication Open to Public Inspection No. 59-27289;  $\text{NaX}'$  (wherein  $\text{X}'$  represents at least one of Cl, Br and I), described in Japanese Patent Publication Open to Public Inspection No. 59-56479;
- (h) transition metals such as V, Cr, Mn, Fe, Co, and Ni, described in Japanese Patent Publication Open to Public Inspection No. 59-56480;  $\text{M}'\text{X}'$ ,  $\text{M}^{II}\text{X}''$ ,  $\text{M}^{III}\text{X}'''$  and A, (wherein  $\text{M}'$  represents at least one alkali metal selected from the group of Li, Na, K, Rb, and Cs;  $\text{M}^{II}$  represents at least one divalent metal selected from the group of Be and Mg;  $\text{M}^{III}$  represents at least one trivalent metal selected from the group of Al, Ga, In, and Tl; A represents a metal oxide;  $\text{X}'$ ,  $\text{X}''$  and  $\text{X}'''$  each represents at least one halogen atom selected from the group of F, Cl, Br, and I), described in Japanese Patent Publication Open to Public Inspection No. 59-75200;
- (i)  $\text{M}'\text{X}'$  (wherein  $\text{M}'$  represents at least one alkali metal selected from the group of Rb or Cs; and  $\text{X}'$  represents at least one halogen atom selected from the group of F, Cl, Br, and I), described in Japanese Patent Publication Open to Public Inspection No. 60-101173;
- (j)  $\text{M}^{II}\text{X}_2'\text{M}^{II}\text{X}_2''$ , (wherein  $\text{M}^{II}$  represents at least an alkaline earth metal selected from the group Ba, Sr, or Ca;  $\text{X}'$  and  $\text{X}''$  each represents at least one halogen atom selected from the group of Cl, Br, or I, and  $\text{X}' \neq \text{X}''$ ), described in Japanese Patent Publication Open to Public Inspection No. 61-23679; and  $\text{LnX}_3''$  (wherein Ln represents at least one rare earth metal selected from the group of Sc, Y, La, Ce, Pr, Nd, Pm, Sm, Gd, Tb, Dy,

## 11

Ho, Er, Tm, Yb, and Lu; X" represents at least one halogen atom selected from the group of F, Cl, Br, and I), described in Japanese Patent Publication Open to Public Inspection No. 61-264084.

(2) Divalent europium activated alkaline earth metal halide phosphor represented by the composition formula of  $M''X_2 \cdot aM''_2 \cdot xEu^{2+}$  (wherein  $M''$  represents at least one alkaline earth metal selected from the group of Ba, Sr, and Ca; X and X' each represent at least one halogen atom selected from the group of Cl, Br, and I; and  $X \neq X'$ ; "a" represents a figure satisfying the relationship of  $0 \leq a \leq 0.1$  and "x" represents a figure satisfying the relationship and  $0 \leq x \leq 0.2$ ), described in Japanese Patent Publication Open to Public Inspection No. 60-84381. Further, said phosphors may comprise additives as described in (a) through (e) below.

(a)  $M'X'$  (wherein  $M'$  represents at least one alkali metal selected from the group of Rb and Cs; X' represents at least one halogen atom selected from the group of F, Cl, Br, and I), described in Japanese Patent Publication Open to Public Inspection No. 60-166379;

(b)  $KX''$ ,  $MgX_2''$  and  $M'''X_3'''$  (wherein  $M'''$  is at least one trivalent metal selected from the group of Sc, Y, La, Gd, and Lu; X'', X''' and X''' each represent at least one halogen atom selected from the group of F, Cl, Br, and I), described in Japanese Patent Publication Open to Public Inspection No. 221483;

(c) B described in Japanese Patent Publication Open to Public Inspection No. 60-228592; oxides such as  $SiO_2$  or  $P_2O_5$ , described in Japanese Patent Publication Open to Public Inspection No. 60-228593;  $LiX''$  and  $NaX''$  (wherein X'' represents at least one halogen atom selected from the group of F, Cl, Br, and I), described in Japanese Patent Publication Open to Public Inspection No. 61-120882;

(d)  $SiO$  described in Japanese Patent Publication Open to Public Inspection No. 61-120883;  $SnX_2''$  (wherein X'' is at least one halogen atom selected from the group of F, Cl, Br, and I), described in Japanese Patent Publication Open to Public Inspection No. 61-120885;

(e)  $CsX''$  and  $SnX_2'''$  (wherein X'' and X''' each represent at least one halogen atom selected from the group of F, Cl, Br, and I), described in Japanese Patent Publication Open to Public Inspection No. 61-235486; and  $CsX''$  and  $Ln^{3+}$  (wherein X'' represents at least one halogen atom selected from the group of F, Cl, Br, and I; Ln represents at least one rare earth element selected from the group of Sc, Y, Ce, Pr, Nd, Sm, Gd, Tb, Dy, Ho, Er, Tm, Yb, and Lu), described in Japanese Patent Publication Open to Public Inspection No. 61-235487.

(3) Rare earth element activated rare earth oxyhalide phosphors represented by the composition formula of  $LnOX:xA$ , (wherein Ln represents at least one of La, Y, Gd, and Lu; X represents at least one of Cl, Br, and I; A represents at least one of Ce and Tb; and "x" represents a figure satisfying the relationship of  $0 < x < 0.1$ ), described in Japanese Patent Publication Open to Public Inspection No. 55-12144;

(4) Cerium activated trivalent metal oxyhalide phosphors represented by the composition formula of  $M''OX:xCe$ , (wherein  $M''$  represents at least one oxidized metal selected from the group of Pr, Nd, Pm, Sm, Eu, Tb, Dy, Ho, Er, Tm, Yb, and Bi; X represents at least one of Cl, Br, and I; "x" represent a figure satisfying the relationship of  $0 < x < 0.1$ ), described in Japanese Patent Publication Open to Public Inspection No. 58-69281;

## 12

(5) Bismuth activated alkali metal halide phosphors represented by the composition formula of  $M'X:xBi$ , (wherein  $M'$  represents at least one alkali metal selected from the group of Rb and Cs; X represents at least one halogen atom selected from the group of Cl, Br, and I; "x" represent a figure satisfying the relationship of  $0 < x \leq 0.2$ ), described in Japanese Patent Application No. 60-70484;

(6) Divalent europium activated alkaline earth metal halophosphate phosphors represented by the composition formula of  $M''_5(PO_4)_3X:Eu^{2+}$ , (wherein  $M''$  represents at least one alkaline earth metal selected from the group of Ca, Sr, and Ba; X represents at least one halogen atom selected from the group of F, Cl, Br, and I; and "x" represents a figure satisfying the relationship of  $0 < x \leq 0.2$ ), described in Japanese Patent Publication Open to Public Inspection No. 60-141783;

(7) Divalent europium activated alkaline earth metal haloborate phosphors represented by the composition formula of  $M''_2BO_3X:xEu^{2+}$  (wherein  $M''$  represents at least one alkaline earth metal selected from the group of Ca, Sr, and Ba; X is at least one halogen atom selected from the group of Cl, Br, and I; and "x" is a figure satisfying the relationship of  $0 < x \leq 0.2$ ), described in Japanese Patent Publication Open to Public Inspection No. 60 157099;

(8) Divalent europium activated alkaline earth metal halophosphate phosphors represented by the composition formula of  $M''_2PO_4X:xEu^{2+}$ , (in which  $M''$  represents at least one alkaline earth metal selected from the group of Ca, Sr, and Ba; X represents at least one halogen atom selected from the group of Cl, Br, and I; and "x" represents a figure satisfying the relationship of  $0 < x \leq 0.2$ ), described in Japanese Patent Publication Open to Public Inspection No. 60-157100;

(9) Divalent europium activated alkaline earth metal hydrogenated halide phosphors represented by the composition formula of  $M''HX:xEu^2$  (wherein  $M''$  represents at least one alkaline earth metal selected from the group of Ca, Sr, and Ba; X represents at least one halogen atom selected from the group of Cl, Br, and I; and "x" represents a figure satisfying the relationship of  $0 < x \leq 0.2$ ), described in Japanese Patent Publication Open to Public Inspection No. 60-217354;

(10) Cerium activated rare earth composite halide phosphors represented by the composition formula of  $LnX_3 \cdot aLn'X_3 \cdot xCe^{3+}$ , (wherein Ln and Ln' each represent at least one rare earth element selected from the group of Y, La, Gd, and Lu; X and X' each represents at least one halogen atom selected from the group of F, Cl, Br, and I;  $X \neq X'$ ; "a" represents a figure satisfying the relationship of  $0 < a \leq 10.0$ ; and "x" represents a figure satisfying the relationship of  $0 < x \leq 0.2$ ), as described in Japanese Patent Publication Open to Public Inspection No. 61-21173;

(11) Cerium activated rare earth composite halide phosphors represented by the composition formula of  $LnX_3 \cdot aM'X':xCe^{3+}$  (wherein Ln represents at least one rare earth element selected from the group of Y, La, Gd, and Lu;  $M'$  represents at least one alkali metal selected from the group of Li, Na, K, Cs, and Rb; X and X' each represents at least one halogen atom selected from the group of Cl, Br, and I; "a" represents a figure satisfying the relationship of  $0 < a \leq 10.0$ ; and "x" represents a figure satisfying the relationship of  $0 < x \leq 0.2$ ), described in JP-A 61-21182;

(12) Cerium activated rare earth halophosphate phosphors represented by the composition formula of  $LnPO_4 \cdot aLnX_3 \cdot xCe^{3+}$  (wherein Ln represents at least one rare earth element selected from the group of Y, La, Gd, and Lu; X represents at least one halogen atom selected from the

## 13

group of F, Cl, Br, and I; "a" represents a figure satisfying the relationship of  $0 < a \leq 10.0$ ; and "x" represents a figure satisfying the relationship of  $0 < x \leq 0.2$ , described in Japanese Patent Publication Open to Public Inspection No. 61-40390;

(13) Divalent europium activated cesium rubidium halide phosphors represented by the composition formula of  $CsX:aRbX':xEu^2$  (wherein X and X' each represents at least one halogen atom selected from the group of Cl, Br, and I; "a" represents a figure satisfying the relationship of  $0 < a \leq 10.0$ ; and "x" represents a figure satisfying the relationship of  $0 < x \leq 0.2$ ), described in Japanese Patent Publication Open to Public Inspection No. No. 61-236888;

(14) Divalent europium activated composite halide phosphors represented by the formula of  $M''X_2.aM'X':xEu^{2+}$  (wherein  $M''$  represents at least one alkaline earth metal selected from the group of Ba, Sr, and Ca;  $M'$  represents at least one alkali metal selected from the group of Li, Rb, and Cs; X and X' each represent at least one halogen atom selected from the group of Cl, Br, and I; "a" represents a figure satisfying the relationship of  $0 < a \leq 10.0$ ; and "x" represents a figure satisfying the relationship of  $0 < x \leq 0.2$ ), described in Japanese Patent Publication Open to Public Inspection No. No. 61-236890.

Of said stimulable phosphors, iodide-containing divalent europium activated alkaline earth metal fluorohalide phosphors, iodide-containing divalent europium activated alkaline earth metal halide phosphors, iodide-containing rare earth element activated rare earth oxyhalide phosphors, and iodide-containing bismuth activated alkaline metal halide phosphors are materials which result in high stimulated luminescence.

Examples used for a support of the present invention are; various types of polymer materials, glass, metals. From the viewpoint of handling information recording materials, flexible sheets or those capable of being machined into a web are suitable. From this viewpoint, preferred are plastic films such as cellulose acetate film, polyester film, polyethylene terephthalate film, polyethylene naphthalate film, polyamide film, polyimide film, triacetate film, and polycarbonate film; metal films of aluminum, iron, copper, and chromium; and metal films coated with hydrophilic fine particles.

Though the thickness of these supports varies depending on the materials used, it is generally from about 3 to about 1,000  $\mu m$ , and from the viewpoint of ease of handling, it is preferably from about 80 to about 500  $\mu m$ .

These supports may have a smooth surface or a matt surface to enhance adhesion with the stimulable phosphor layer.

These supports may be provided with a sublayer in order to improve the adhesion property of a stimulable phosphor layer between a surface of the support.

Examples of binders employed in said sublayer include proteins such as gelatin, polysaccharides such as dextran, natural polymers such as gum Arabic, and synthetic polymers such as polyvinyl butyral, polyvinyl acetate, nitrocellulose, ethylcellulose, vinylidene chloride-vinyl chloride copolymers, polyalkyl acrylate, polyalkyl methacrylate), vinyl chloride-vinyl acetate copolymers, polyurethane, cellulose acetate butyrate, polyvinyl alcohol, and linear polyesters. Further, these binders may be subjected to cross-linking employing bridging agents.

Examples of binders employed in said stimulable phosphor layer include compounds described for binders of the sublayer. These binders may also be subjected to cross-linking employing bridging agents.

Preferred weight ratio of a binder to said stimulable phosphor in the coating composition varies depending on the

## 14

properties and the kinds of the targeted radiation image conversion panel. Usually, the preferred weight ratio of the binder to the stimulable phosphor is 1 to 20. In order to get larger brightness and higher sharpness of the radiation image conversion panel, the amount of binder is preferably smaller, and by consideration of easiness of coating, more preferred ratio of the binder to the stimulable phosphor is 2 to 10.

Listed as examples of solvents, employed to prepare said stimulable phosphor layer 4 coating composition, are lower alcohols such as methanol, ethanol, isopropanol, and n-butanol; ketones such as acetone, methyl ethyl ketone, methyl isobutyl ketone, and cyclohexanone; esters of lower fatty acids and lower alcohols such as methyl acetate, ethyl acetate, and n-butyl acetate; ethers such as dioxane, ethylene glycol monoethyl ether and ethylene glycol monomethyl ether; aromatic compounds such as toluene and xylene; halogenated hydrocarbons such as methylene chloride and ethylene chloride; and mixtures thereof.

Further, various additives such as dispersing agents to enhance the dispersion of said stimulable phosphors in said coating composition, and plasticizers to enhance a bonding force between binders and phosphors in the resulting stimulable phosphor layer may be incorporated into said coating composition. Listed as examples of dispersing agents employed for said purpose may be phthalic acid, stearic acid, caproic acid, and oleophilic surface active agents. Listed as examples of plasticizers are phthalic acid esters such as triphenyl phosphate, cresyl phosphate, and diphenyl phosphate; phthalic acid esters such as dimethoxyethyl phthalate; glycolic acid esters such as ethyl phthalyl ethyl glycolate and butyl phthalyl butyl glycolate; polyesters of polyethylene glycol with aliphatic dibasic acids such as polyester of triethylene glycol with adipic acid and polyester of diethylene glycol with succinic acid.

A stimulable phosphor layer coating composition is prepared employing any of the common homogenizers such as a ball mill, a sand mill, an attritor, a three-pole mill, a high-speed impeller homogenizer, a Kady mill, and an ultrasonic homogenizer.

The coating composition prepared as above is uniformly coated onto the surface of the sublayer, whereby a coating composition layer is formed. Said coating is carried out employing conventional coating means such as a doctor blade, a roll coater, a knife coater, a comma coater, and a lip coater. The resulting coating is dried through gradual heating, whereby the formation of said stimulable phosphor layer 4 on the sublayer is completed.

The thickness of said stimulable phosphor layer varies depending on the target characteristics of the radiation image conversion panel, the types of stimulable phosphors, and the mixing ratio of binders to stimulable phosphors. However, said thickness is preferably in the range of 10 to 1,000  $\mu m$ , and is more preferably in the range of 10 to 500  $\mu m$ .

A phosphor sheet, prepared by applying the stimulable phosphor layer onto a support, is then cut into specified sizes. Any of several common methods may be employed for cutting. However, from the viewpoint of workability as well as accuracy, trimming machines or punching machines are preferred.

The radiation image conversion panel of the present invention is preferably provided with a protective layer (hereinafter occasionally referred to as a protective film) in order to chemically and physically protect the surface of the stimulable phosphor layer. Said protective layer may be suitably constituted based on its purposes as well as its use.

Examples of protective layers to cover said stimulable phosphor layer may be polyester film, polymethacrylate

film, nitrocellulose film, and cellulose acetate film, provided with a stimulating light absorbing layer at a haze ratio of 5 to 60 percent, determined by the method described in ASTMD-1003. Of these, from the viewpoint of transparency as well as strength, stretched films such as polyethylene terephthalate film and polyethylene naphthalate film are preferred, and from the aspect of moisture resistance, metalized films are specifically preferred, which are obtained by applying a thin layer comprised of metal oxides or silicone nitride onto said polyethylene terephthalate film or polyethylene naphthalate film through vacuum evaporation.

The haze ratio to obtain the effects of the present invention is preferably from 5 to 60 percent, and is more preferably from 10 to 50 percent. A haze ratio of less than 5 percent is not preferred, since effects to minimize image unevenness, as well as to minimize linear noise, decrease. On the other hand, said haze ratio of more than or equal to 60 percent is also not preferred, since sharpness enhancing effects are degraded.

In order to satisfy required moisture resistance, optimal moisture resistance is obtained by laminating a plurality of resinous films and metalized films obtained by vacuum-evaporating metal oxides onto said resinous film. In order to minimize degradation of stimulable phosphors due to moisture absorption, it is preferable to achieve no more than 50 g/m<sup>2</sup>·day. The method of laminating a resinous film is not specially limited and known conventional methods can be applied.

Further, an excitation light absorbing layer is preferably provided between the laminated resinous films so that said excitation light absorbing layer is protected from physical impact as well as chemical modification so as to stabilize the plate functions over an extended period of time. In addition, said excitation light absorbing layer may be provided in a plurality of positions, and an adhesive layer for lamination may be comprised of coloring agents, thereby being utilized as the excitation light absorbing layer.

A protective film may be provided a adhesion layer between a stimulable phosphor layer. However, a structure which covers all of the stimulable phosphor surface is preferred. This structure is called a "sealed structure". When a phosphor plate is sealed employing a protective film, it is possible to employ any of the several conventionally known methods such as a phosphor sheet which is interposed between moisture resistant protective films and the peripheral edge of which is subjected to lamination under application of heat and pressure employing an impulse sealer, and lamination is carried out between rollers under application of heat and pressure. By employing a heat fusible resinous film as the resinous layer of the outermost layer in contact with the phosphor sheet of the moisture resistant protective film, the moisture resistant protective film is fused, whereby the efficiency of sealing work of the phosphor sheets is enhanced. The moisture resistant protective film is preferably provided on both sides of the phosphor sheet and the peripheral edge of said moisture resistant protective films, which is located beyond the peripheral edge of said phosphor sheet, is fused to result in a sealed structure, whereby it is possible to prevent infusion of water from the outside. Further, the moisture resistant protective film on one side of the support may be laminated with at least one aluminum film. By employing such a support, it is possible to assure minimal water infusion.

Further, said heat fusion, which is carried out employing an impulse sealer, is preferably performed under reduced pressure to minimize the displacement of the phosphor sheet in the moisture resistant protective film and to remove moisture from the atmosphere.

Still further, the phosphor surface may or may not be allowed to come into contact with the heat fusible resinous layer of the outermost layer on the side in contact with the phosphor surface of the moisture resistant protective film. 5 The non-contact state, as described herein, refers to the state in which the phosphor surface and the moisture resistant protective film are optically and mechanically handled mostly as discontinuous body, even though they may come into "point" contact. Further, the heat fusible film, as 10 described herein, refers to the resinous films which are fusible in the generally used impulse sealer, and include, for example, ethylene-vinyl acetate copolymers (EVA), polypropylene (PP) film, and polyethylene (PE) film. However, the present invention is not limited to these 15 examples.

The radiation image capturing method according to one of the embodiments is characterized in X-rays are irradiated onto the stimulable phosphor layer from the support side of said radiation image conversion panel, and output image information is read from the side of said stimulable phosphor layer.

FIG. 2 shows one example of a radiation image conversion method employing a radiation image conversion panel. The radiation image conversion panel of the present invention is advantageously employed based on the radiation image conversion method schematically shown in FIG. 2. 25 Namely, in FIG. 2, numeral 21 is a radiation generating unit, 22 is the image subject, 23 is the radiation image conversion panel according to the present invention, 24 is a stimulating 30 excitation light source, 25 is a photoelectric transfer unit which detects the stimulated luminescence emitted from said conversion panel, 26 is a unit which reproduces images based on signals detected by 25, 27 is a unit to display the 35 reproduced images, 28 is a filter which transmits only stimulated phosphorescence upon separating said stimulating excitation light and the stimulated phosphorescence. Incidentally, units described by numerals 25 and higher are 40 not particularly limited as above, as long as they can reproduce images based on light information from 23, utilizing any suitable method.

As shown in FIG. 2, radiation R from radiation generating unit 21 is incident (RI) onto the support side of radiation image conversion panel 23 while transmitting subject 22. The resulting incident radiation RI is absorbed by the 45 stimulable phosphor layer of said radiation image conversion panel 23 and energy thereof is accumulated so that an accumulated image of the radiation transmission image is formed.

Subsequently, said accumulated image is excited employing a stimulating excitation light from stimulating excitation light source 24, and the accumulated energy is released as 50 stimulated luminescence.

The intensity of said stimulated luminescence is proportional to the amount of the accumulated radiation energy. 55 The resulting light signals are subjected to photoelectric transfer employing photoelectric transfer unit 25 such as a photomultiplier tube, and images are reproduced by image reproducing unit 26. The reproduced images are displayed onto image display unit 27. Thus, it is possible to observe the 60 radiation transmission image of said subject.

In the system in which X-rays are incident onto the phosphor layer side and reading is carried out on the phosphor side, subject images such as a human body are present on the phosphor layer side. Therefore, reading is generally carried out at other locations utilizing a cassette type or by conveying the panel itself. Accordingly, when such a system is employed, it takes time between the 65

imaging and the reading. As a result, it is impossible to carry out mass medical examinations during a short period of time. On the other hand, in the system described above, in which X-rays are incident on the rear side and reading is carried out on the front side, reading is immediately carried out without need for moving the panel. As a result, said system exhibits advantages in which many subjects can be imaged during a short period of time.

### EXAMPLES

The present invention will now be described with reference to examples. However, the present invention is not to be construed as being limited to these examples.

#### Example 1

##### Preparation of Radiation Image Conversion Panels

###### Preparation of Radiation Image Conversion Panel 1

###### Preparation of Phosphors

The stimulable phosphor precursor of europium activated barium fluoride iodide was synthesized as follows. Charged into a reaction vessel were 2,780 ml of an aqueous  $\text{BaI}_2$  solution (3.6 mol/L) and 27 ml of an aqueous  $\text{EuI}_3$  solution (0.15 mol/L). While stirring, the reaction mother solution in said reaction vessel was maintained at 83° C. Subsequently, 322 ml of an aqueous ammonium fluoride solution (8 mol/liter) were poured into said mother solution employing a roller pump, whereby precipitates were formed. After pouring, the resulting precipitates underwent ripening for 2 hours, while stirring and maintaining said temperature. Subsequently, the resulting precipitates were collected through filtration, washed with ethanol, and dried, whereby europium activated barium fluoride iodide crystals were obtained. In order to minimize the variation of particle size distribution due to calcination during sintering, ultra-fine alumina particle powder was added in an amount of 0.2 percent by weight, and the resulting mixture was well stirred so that said ultra-fine alumina particle powder was uniformly adhered onto the surface of said crystals. A quartz boat was filled with the resulting mixture and calcined under an atmosphere of hydrogen gas at 850° C. for 2 hours in a tube furnace. Thereafter, the resulting product was classified, whereby europium activated barium fluoride iodide phosphor particles, having an average particle diameter of 4  $\mu\text{m}$ , were prepared.

###### Preparation of Phosphor Layer Coating Composition

Added to a methyl ethyl ketone-toluene (1:1) solvent mixture were 100 g of the phosphor prepared as above and

16.7 g of a polyester resin (Biron 63SS, 30 percent solids, manufactured by Toyobo Co.), and the resulting mixture was dispersed employing a propeller mixer. Subsequently, the viscosity was adjusted to 25 to 30 Pa·s, whereby a phosphor layer coating composition was prepared.

###### Preparation of Phosphor Sheet 1

The phosphor layer coating composition prepared as above was applied onto a 250  $\mu\text{m}$  thick polyethylene terephthalate support, employing a doctor blade, so as to obtain a coating width of 1,000 mm and a coating thickness of 230  $\mu\text{m}$ . Thereafter, the resultant coating was dried at 100° C. for 15 minutes, whereby phosphor layer 1 was formed, which was designated as Phosphor Sheet 1.

###### Preparation of Phosphor Sheet 2

15 Phosphor Sheet 2 was prepared in the same manner as said Phosphor Sheet 1, except that after coating said phosphor layer, a compression treatment was carried out employing the method described below.

###### Compression Treatment of Phosphor Sheet 2

20 After coating and drying said phosphor layer, a compression treatment was carried out employing a group of rollers constituted as shown in FIG. 1.

A compression section was comprised of three rollers in series, and two nips were formed between heating rollers 9-1 and 9-3, and compliant roller 9-2. In addition, adjustment was carried out so that said compliant roller came into contact only with the phosphor layer forming surface.

25 Employed as said heating rollers 9-1 and 9-3 were ones having a diameter of 300 mm $\phi$  and a surface of 0.2S. Employed as said compliant roller 9-2 was polyester Mirrortex Roll (manufactured by Yamauchi Gomu), having a diameter of 250 mm $\phi$ , a Shore D hardness of D75 degrees, a crown length of 0  $\mu\text{m}$ , and a center-line mean surface roughness Ra of 0.4  $\mu\text{m}$ , specified by JIS B 0601. Further, said compression treatment was carried out in such a manner that the temperature of said heating rollers was set at 70° C. and the linear pressure was adjusted to 1 kN/cm.

###### Preparation of Phosphor Sheets 3 through 18

30 40 Phosphor Sheets 3 through 18 were prepared in the same manner as Phosphor Sheet 2, except that the Shore hardness, materials, the center-line mean surface roughness Ra, the crown length, and compression conditions (heating temperature and linear pressure) of said compliant roller were varied as described in Table 1.

TABLE 1

| Radiation Image Conversion Panel No. | Compression Treatment | Characteristics of Compliant Roller |                 |                                       |                                  | Compression Condition |                            | Remarks |
|--------------------------------------|-----------------------|-------------------------------------|-----------------|---------------------------------------|----------------------------------|-----------------------|----------------------------|---------|
|                                      |                       | Roller Hardness (in degrees)        | Roller Material | Surface Roughness (in $\mu\text{m}$ ) | Crown Length (in $\mu\text{m}$ ) | Temperature (in ° C.) | Linear Pressure (in kN/cm) |         |
| 1                                    | not carried out       | —                                   | —               | —                                     | —                                | —                     | —                          | Comp.   |
| 2                                    | carried out           | 75                                  | polyester resin | 0.4                                   | 0                                | 70                    | 1                          | Comp.   |
| 3                                    | carried out           | 85                                  | polyester resin | 0.3                                   | 0                                | 70                    | 1                          | Comp.   |
| 4                                    | carried out           | 90                                  | polyester resin | 0.3                                   | 0                                | 70                    | 1                          | Comp.   |
| 5                                    | carried out           | 95                                  | polyester resin | 0.2                                   | 0                                | 70                    | 1                          | Inv.    |
| 6                                    | carried out           | 99                                  | polyester resin | 0.2                                   | 0                                | 70                    | 1                          | Comp.   |
| 7                                    | carried out           | 100 or more                         | steel           | 0.05                                  | 0                                | 70                    | 1                          | Comp.   |

TABLE 1-continued

| Radiation<br>Image<br>Conversion<br>Panel No. | Compression<br>Treatment | Characteristics of Compliant Roller   |                    |                                                  | Compression<br>Condition               |                                               |                                     | Remarks |
|-----------------------------------------------|--------------------------|---------------------------------------|--------------------|--------------------------------------------------|----------------------------------------|-----------------------------------------------|-------------------------------------|---------|
|                                               |                          | Roller<br>Hardness<br>(in<br>degrees) | Roller<br>Material | Surface<br>Rough-<br>ness<br>(in $\mu\text{m}$ ) | Crown<br>Length<br>(in $\mu\text{m}$ ) | Temper-<br>ature<br>(in $^{\circ}\text{C}$ .) | Linear<br>Pressure<br>(in<br>kN/cm) |         |
| 8                                             | carried out              | 75                                    | polyester<br>resin | 0.3                                              | 0                                      | 40                                            | 1                                   | Inv.    |
| 9                                             | carried out              | 75                                    | polyester<br>resin | 0.3                                              | 0                                      | 140                                           | 1                                   | Inv.    |
| 10                                            | carried out              | 75                                    | polyester<br>resin | 0.3                                              | 0                                      | 160                                           | 1                                   | Inv.    |
| 11                                            | carried out              | 75                                    | polyester<br>resin | 0.3                                              | 0                                      | 70                                            | 0.4                                 | Inv.    |
| 12                                            | carried out              | 75                                    | polyester<br>resin | 0.3                                              | 0                                      | 70                                            | 2.5                                 | Inv.    |
| 13                                            | carried out              | 75                                    | polyester<br>resin | 0.3                                              | 0                                      | 70                                            | 3.5                                 | Inv.    |
| 14                                            | carried out              | 75                                    | polyester<br>resin | 0.3                                              | 5                                      | 70                                            | 1                                   | Inv.    |
| 15                                            | carried out              | 75                                    | polyester<br>resin | 0.3                                              | 30                                     | 70                                            | 1                                   | Inv.    |
| 16                                            | carried out              | 75                                    | polyester<br>resin | 0.3                                              | 150                                    | 70                                            | 1                                   | Inv.    |
| 17                                            | carried out              | 75                                    | polyester<br>resin | 0.3                                              | 800                                    | 70                                            | 1                                   | Inv.    |
| 18                                            | carried out              | 75                                    | polyester<br>resin | 0.3                                              | 1300                                   | 70                                            | 1                                   | Inv.    |

Inv.: Present Invention, Comp.: Comparative Example

## Preparation of Moisture Resistant Protective Film

Employed as a protective film on the phosphor layer coated side of phosphor sheets **1** through **18**, prepared as above, was one comprised of Configuration (A) described below.

## Configuration (A)

NY15///VMPET12//VMPET12//PET12//CPP20

NY: nylon

PET: polyethylene terephthalate

CPP: casting polypropylene

VMPET: alumina vacuum-evaporated PET (being a commercially available product, manufactured by Toyo Metalizing Co.)

The numeral shown following each resinous film is the thickness (in  $\mu\text{m}$ ) of each resinous layer.

Said "///" refers to a dry lamination adhesion layer in which the thickness of the coloring agent layer is 3.0  $\mu\text{m}$ . Employed as an adhesive for said dry lamination was a 2-liquid reaction type urethane based adhesive.

Further, employed as a protective film on the rear surface of the support of the phosphor sheet was a dry laminate film composed of a CPP 30  $\mu\text{m}$ /aluminum film 9  $\mu\text{m}$ /polyethylene terephthalate (PET) 188  $\mu\text{m}$ . Further, in said configuration, the thickness of the adhesive layer was 1.5  $\mu\text{m}$  and a 2-liquid reaction type urethane based adhesive was employed.

## Preparation of Radiation Image Conversion Panel

Each of Phosphor Sheets **1** through **18** was cut into 20 $\times$ 20 cm square sheets. Subsequently, the periphery of the resultant sheet was fuse-sealed with the moisture resistant protective film prepared as above under reduced pressure, employing an impulse sealer, whereby radiation image conversion panels **1** through **18** were prepared. Incidentally, fusing was carried out so that the distance from the fused section to the periphery of said phosphor sheet was 1 mm. A 3 mm wide impulse heater was employed for said fusing.

<sup>30</sup>  
Evaluation of Radiation Image Conversion Panels  
Employing each of the radiation image conversion panels or the phosphor sheets prepared as above, the filling ratio, the luminance, and the sharpness, as well as its fluctuation, were evaluated based on the methods described below.

## 35 Measurement of Phosphor Filling Ratio

The protective layer of each phosphor sheet was peeled off and removed. Subsequently, employing methyl ethyl ketone, the phosphor layer was peeled off or dissolved out, filtered and dried. The resultant phosphor was burned at 600  $^{\circ}\text{C}$ . for one hour employing an electric furnace, so as to remove the surface resin on the phosphor. The phosphor filling ratio was then calculated based on the formula described below.

<sup>40</sup>  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
72

## Evaluation of Sharpness

Said sharpness was determined as described below. In regard to each of the radiation image conversion panels, the rear surface of the support of the phosphor sheet was exposed to X-rays at a tube voltage of 80 kVp through a lead MTF chart. Thereafter, said panel was subjected to excitation by operating a He-Ne laser beam. Stimulated luminescence, emitted from the phosphor layer, was received by the same light receiving unit, as described above, and was converted into electrical signals, which were subjected to analogue/digital conversion and recorded onto a magnetic tape. Information on the resultant magnetic tape was analyzed utilizing a computer, and the modulation transfer function (MTF) in 1 cycle/mm of an X-ray image recorded in said magnetic tape was examined. Said measurement was carried out at 25 positions on said radiation image conversion panel. The resultant average (being the average MTF) was defined as sharpness, which was expressed utilizing a relative value, when the sharpness of Radiation Image Conversion panel 1 was deemed to be 100.

## Evaluation of Sharpness Fluctuation

In the 1,000 mm wide length of the compliant roll employed for the preparation, 25 positions were randomly chosen, and the MTF of each position was determined based on the same method as said sharpness evaluation method. The maximum and minimum values were obtained from the resultant MTF values, and the sharpness fluctuation was calculated based on the formula shown below.

$$\text{Sharpness fluctuation} = (\text{maximum MTF value} - \text{minimum MTF value}) / \text{average MTF value} (\text{in percent})$$

Table 2 shows the obtained results.

TABLE 2

| Radiation | Evaluation Result          |                      |                    |                    |                              |         |
|-----------|----------------------------|----------------------|--------------------|--------------------|------------------------------|---------|
|           | Image Conversion Panel No. | Filling ratio (in %) | Relative Luminance | Relative Sharpness | Sharpness Fluctuation (in %) | Remarks |
| 1         | 52                         | 100                  | 100                | 2.5                | Comp.                        |         |
| 2         | 54                         | 100                  | 102                | 5.3                | Comp.                        |         |
| 3         | 59                         | 102                  | 106                | 1.3                | Inv.                         |         |
| 4         | 61                         | 102                  | 112                | 1.0                | Inv.                         |         |
| 5         | 63                         | 103                  | 113                | 1.4                | Inv.                         |         |
| 6         | 63                         | 93                   | 113                | 3.4                | Comp.                        |         |
| 7         | 65                         | 88                   | 114                | 4.7                | Comp.                        |         |
| 8         | 55                         | 100                  | 105                | 1.9                | Inv.                         |         |
| 9         | 62                         | 102                  | 113                | 1.1                | Inv.                         |         |
| 10        | 62                         | 102                  | 112                | 1.7                | Inv.                         |         |
| 11        | 56                         | 100                  | 105                | 1.5                | Inv.                         |         |
| 12        | 64                         | 100                  | 114                | 1.0                | Inv.                         |         |
| 13        | 65                         | 99                   | 115                | 1.8                | Inv.                         |         |
| 14        | 61                         | 102                  | 112                | 0.9                | Inv.                         |         |
| 15        | 62                         | 102                  | 113                | 0.7                | Inv.                         |         |
| 16        | 62                         | 102                  | 111                | 0.4                | Inv.                         |         |
| 17        | 61                         | 102                  | 112                | 0.8                | Inv.                         |         |
| 18        | 61                         | 102                  | 112                | 1.1                | Inv.                         |         |

Inv.: Present Invention, Comp.: Comparative Example

As can clearly be seen from Table 2, it was confirmed that by carrying out a compression treatment, employing a compliant roller having a crown length as well as having a Shore hardness according to the present invention, it was possible to enhance the stimulable phosphor filling ratio to achieve high luminance as well as high sharpness, and in addition, to decrease the sharpness fluctuation of the radiation image conversion panels. Further, it was revealed that by providing the conditions specified in claims 3 and 4 of the present invention, said effects were further enhanced.

## Example 201

Preparation of Radiation Image Conversion Panels  
Preparation of Radiation Image Conversion Panel 1  
Preparation of Phosphors

5 The stimulable phosphor precursor of europium activated barium fluoride iodide was synthesized as follows. Charged into a reaction vessel were 2,780 ml of an aqueous  $\text{BaI}_2$  solution (3.6 mol/L) and 27 ml of an aqueous  $\text{EuI}_3$  solution (0.15 mol/L). While stirring, the reaction mother solution in 10 said reaction vessel was maintained at 83° C. Subsequently, 322 ml of an aqueous ammonium fluoride solution (8 mol/liter) were added to said mother solution employing a roller pump, whereby precipitates were formed. After the 15 addition, the resulting precipitates underwent ripening for 2 hours while stirred at the stated temperature. Subsequently, the resulting precipitates were collected through filtration, washed with ethanol, and dried, whereby europium activated barium fluoride iodide crystals were obtained. In order to 20 minimize variation of particle size distribution due to calcination during sintering, ultra-fine alumina powder particles were added in an amount of 0.2 percent by weight, and the resulting mixture was well stirred so that said ultra-fine alumina powder particles were uniformly adhered onto the surface of said crystals. A quartz boat was filled with the 25 resulting mixture and calcined under an atmosphere of hydrogen gas at 850° C. for 2 hours in a tube furnace. Thereafter, the resulting product was classified, whereby europium activated barium fluoride iodide phosphor particles, having an average particle diameter of 4  $\mu\text{m}$ , were 30 prepared.

## Preparation of Phosphor Layer Coating Composition

Added to a methyl ethyl ketone-toluene (1:1) solvent mixture were 100 g of the phosphor prepared as above, and 16.7 g of a polyester resin (30 percent solids) having a Tg of 35 45° C., and the resulting mixture was dispersed employing a propeller mixer. Subsequently, the viscosity was adjusted to 25 to 30 Pa·s, whereby a phosphor layer coating composition was prepared.

## Preparation of Phosphor Sheet 1

40 The phosphor layer coating composition prepared as above was applied, employing a doctor blade, onto a 250  $\mu\text{m}$  thick polyethylene terephthalate support having a Tg of 69° C. so as to obtain a coating width of 1,000 mm and a coating thickness of 230  $\mu\text{m}$ . Thereafter, the resultant coating was 45 dried at 100° C. for 15 minutes, whereby phosphor layer 1 was formed. Thereafter, the coating was subjected to compression treatment employing the method described below, whereby Phosphor Sheet 1 was prepared.

## Compression Treatments

50 After coating and drying said phosphor layer, compression treatment was carried out employing a group of rollers constituted as shown in FIG. 1.

A compression section was comprised of three rollers in series, and two nips were formed between heating rollers 9-1 and 55 9-2, and compliant roller 9-2, and compliant roller 9-2. In addition, adjustment was carried out so that said compliant roller came into contact only with the phosphor layer forming surface.

Employed as said heating rollers 9-1 and 9-3 were ones having a diameter of 300 mm $\phi$  and a surface of 0.2S.

60 Employed as said polyester compliant roller 9-2 was Mirrortex Roll (manufactured by Yamauchi Gomu), having a diameter of 250 mm $\phi$ , a hardness of Shore D 75 degrees, and a center-line mean surface roughness Ra of 0.4  $\mu\text{m}$ , specified by JIS B 0601. Further, said compression treatment was 65 carried out in such a manner that the temperature of said heating rollers was set at 40° C. and the linear pressure was adjusted to 1 kN/cm.

## Preparation of Phosphor Sheets 2 Through 12

Phosphor Sheets 2 through 12 were prepared in the same manner as Phosphor Sheet 1, except that the types (Tg was 10° C., 5° C., -20° C., and -40° C.) and compression conditions (applied pressure, temperature, and linear pressure) were varied to those described in Table 201.

## Preparation of a Moisture Resistant Protective Film

Employed as a protective film on the phosphor layer coated side of Phosphor Sheets 1 through 12, prepared as above, was one comprised of Configuration (A) described below.

## Configuration (A)

NY15///VMPET12///VMPET12//PET12//CPP20

NY: nylon

PET: polyethylene terephthalate

CPP: casting polypropylene

VMPET: alumina vacuum-evaporated PET (being a commercially available product, manufactured by Toyo Metalizing Co.)

The numeral shown following each resinous film is the thickness (in  $\mu\text{m}$ ) of each resinous layer.

Said "///" refers to the dry lamination adhesion layer in which the thickness of the coloring agent layer is 3.0  $\mu\text{m}$ . Employed as an adhesive for said dry lamination was a 2-liquid reaction type urethane based adhesive.

Further, employed as a protective film on the rear surface of the support of the phosphor sheet was a dry laminate film composed of a 30  $\mu\text{m}$  CPP/9  $\mu\text{m}$  aluminum film/188  $\mu\text{m}$  polyethylene terephthalate (PET). Further, in said configuration, the thickness of the adhesive layer was 1.5  $\mu\text{m}$  and a 2-liquid reaction type urethane based adhesive was employed.

## Preparation of Radiation Image Conversion Panel

Each of Phosphor Sheets 1 through 12 was cut into 20×20 cm square sheets. Subsequently, the periphery of the resultant sheet was fuse-sealed with the moisture resistant protective film, prepared as above, under reduced pressure, employing an impulse sealer, whereby radiation image conversion panels 1 through 18 were prepared. Incidentally, fusing was carried out so that the distance from the fused section to the periphery of said phosphor sheet was 1 mm. A 3 mm wide impulse heater was employed for said fusing.

## Evaluation of Radiation Image Conversion Panels

Employing each of the radiation image conversion panels prepared as above, sharpness as well as its fluctuation and image unevenness were evaluated based on the methods described below.

## Evaluation of Sharpness

Said sharpness was determined as described below. In regard to each of the radiation image conversion panels, the rear surface of the support of the phosphor sheet was exposed to X-rays at a tube voltage of 80 kVp through a lead MTF chart. Thereafter, said panel was subjected to excitation by operating a He-Ne laser beam. Stimulated luminescence, emitted from the phosphor layer, was received by the same light receiving unit, as described above, and was converted into electrical signals, which were subjected to analogue/digital conversion and recorded onto a magnetic tape. Information on the resultant magnetic tape was analyzed utilizing a computer, and the modulation transfer function (MTF) in 1 cycle/mm of an X-ray image recorded in said magnetic tape was examined. Said measurement was carried out at 25 positions on said radiation image conversion panel. The resultant average (being the average MTF) was defined as sharpness, which was expressed utilizing a relative value, when the sharpness of Radiation Image Conversion Panel 1 was deemed to be 100.

## Evaluation of Sharpness Fluctuation

In each of the radiation image conversion panels, 25 positions were randomly chosen, and the MTF of each position was determined based on the same method as said sharpness evaluation method. The maximum and minimum values were obtained from the resultant MTF values, and the sharpness fluctuation was calculated based on the formula shown below.

$$\text{Sharpness fluctuation} = (\text{maximum MTF value} - \text{minimum MTF value}) / \text{average MTF value} (\text{in percent})$$

Table 2 shows the obtained results.

## Evaluation of Image Unevenness

Each of the radiation image conversion panels was exposed to X-rays at a tube voltage of 80 kVp. Thereafter, said panel was scanned employing a He-Ne laser beam (633 nm) and then excited. Stimulated luminescence, emitted from the phosphor layer, was received by a receiving unit (a

TABLE 201

| Radiation Image Conversion Panel No. | Tg of Polymer | Compression Condition            |                      |                                                                                |                    |                              |                       | Remarks |
|--------------------------------------|---------------|----------------------------------|----------------------|--------------------------------------------------------------------------------|--------------------|------------------------------|-----------------------|---------|
|                                      |               | Resin of Phosphor Layer (in °C.) | Temperature (in °C.) | Linear Pressure (in kN/cm)                                                     | Relative Sharpness | Sharpness Fluctuation (in %) | Image Unevenness Rank |         |
| 1                                    | 45            | 40                               | 1                    | 100                                                                            | 3.4                | 3                            | Comp.                 |         |
| 2                                    | 45            | 100                              | 1                    | 103                                                                            | 5.2                | 4                            | Comp.                 |         |
| 3                                    | 10            | 40                               | 1                    | 101                                                                            | 1.9                | 2                            | Comp.                 |         |
| 4                                    | 10            | 100                              | 1                    | 104                                                                            | 4.9                | 4                            | Comp.                 |         |
| 5                                    | 5             | 40                               | 1                    | 109                                                                            | 0.9                | 1                            | Inv.                  |         |
| 6                                    | -20           | —                                | —                    | 95                                                                             | 6.4                | 5                            | Comp.                 |         |
| 7                                    | -20           | 20                               | 1                    | 113                                                                            | 0.4                | 0                            | Inv.                  |         |
| 8                                    | -20           | 40                               | 1                    | 115                                                                            | 0.3                | 0                            | Inv.                  |         |
| 9                                    | -20           | 100                              | 1                    | 116                                                                            | 4.9                | 4                            | Comp.                 |         |
| 10                                   | -20           | 40                               | 0.4                  | 113                                                                            | 1.3                | 2                            | Inv.                  |         |
| 11                                   | -20           | 40                               | 6                    | 116                                                                            | 1.7                | 2                            | Inv.                  |         |
| 12                                   | -40           | 40                               | 1                    | impossible to evaluate due to roller adhesion during the compression treatment |                    |                              | Comp.                 |         |

## 25

photomultiplier having a spectral sensitivity of S-5) and was converted into electrical signals, which were reproduced as images employing an image reproduction unit and then were printed out while enlarging by a factor of two. Subsequently, the resulting prints were visually observed and the occurrence of image unevenness was evaluated. Said image unevenness was evaluated based on 6-rank from 0 to 5 according to the criteria described below.

0: no image unevenness was noticed

1: image unevenness was noticed in 1 or 2 positions on the image

2: image unevenness was noticed in 3 or 4 positions on the image

3: image unevenness was noticed in 3 or 4 positions on the image and high density image unevenness was noticed in 1 or 2 positions among them

4: image unevenness was noticed in at least 5 positions on the image

5: high density image unevenness was noticed in at least 5 positions on the image.

Table 201 also shows the obtained results as above.

As can clearly be seen from Table 201, the following was confirmed. When the stimulable phosphor layer, according to the present invention, comprised a polymer resin, having a glass transition point (Tg) of -30 to 5°C., in an amount of 50 percent by weight based on the total polymer resins of said stimulable phosphor layer, and the phosphor sheet was subjected to compression treatment in the temperature range of at least the Tg of said polymer resin to at most the Tg of the support, smoothness of said stimulable phosphor layer was improved. It was possible to obtain high sharpness and also to decrease the sharpness fluctuation as well as the image unevenness. Further, it was found that by practicing the linear pressure conditions specified in claim 2 of the present invention, the resultant effects were more pronounced.

According to the present invention, it is possible to provide a radiation panel which exhibits excellent sharpness as well as minimal image evenness, a production method thereof, and a radiation image capturing method using the same.

What is claimed is:

1. A method for preparing a radiation image conversion panel, which comprises the steps of:

(a) applying onto a support a stimulable phosphor coating composition comprising a stimulable phosphor and a polymer resin to form a stimulable phosphor layer;

(b) drying the stimulable phosphor layer; and

(c) subjecting the stimulable phosphor layer on the support to a compression treatment employing a calender roller which comes into contact with the stimulable phosphor layer to form the radiation image conversion panel, wherein the calender roller has a crown value of 10 to 1,000  $\mu\text{m}$ .

2. The method for preparing a radiation image conversion panel of claim 1, wherein the polymer resin in the step (a) comprises a polymer having a glass transition point of not more than 5°C. and not less than -30°C. and the polymer accounts for at least 50 weight % of the polymer resin in the stimulable phosphor layer; and the temperature of the calender roller in the step (c) is not less than the glass transition point of the polymer resin acid not more than a glass transition point of the support.

## 26

3. The method for preparing a radiation image conversion panel of claim 1, wherein the compression treatment in the step (c) is carried out at a pressure of 500 to 5,000 N/cm and at a temperature of 50 to 150°C.

4. The method for preparing a radiation image conversion panel of claim 1, wherein the calender roller in the step (c) has a center-line mean surface roughness Ra of 0.05 to 3  $\mu\text{m}$ .

5. The radiation image conversion panel prepared according to the method of claim 1.

6. The radiation image conversion panel of claim 5, wherein the stimulable phosphor incorporated in the stimulable phosphor layer is an Eu added BaFI compound.

7. A method for capturing a radiation image, which comprises the steps of:

(a) irradiating the radiation image conversion panel of claim 5 from the support side of the radiation image conversion panel with X-ray which passes through an object being diagnosed so that to store a radiation energy;

(b) stimulating the stimulable layer with an electromagnetic wave to produce stimulated luminescence; and

(c) reading the stimulated luminescence from the stimulable phosphor layer side.

8. A method for preparing a radiation image conversion panel, which comprises the steps of:

(a) applying onto a support a stimulable phosphor coating composition comprising a stimulable phosphor and a polymer resin to form a stimulable phosphor layer;

(b) drying the stimulable phosphor layer; and

(c) subjecting the stimulable phosphor layer on the support to a compression treatment employing a calender roller which comes into contact with the stimulable phosphor layer to form the radiation image conversion panel, wherein the calender roller comprises a resin and the surface of the calender roller has a Shore D hardness of D80 to D97° and wherein the calender roller in the step (c) has a center-line mean surface roughness Ra of 0.05 to 3  $\mu\text{m}$ .

9. A method for preparing a radiation image conversion panel, which comprises the steps of:

(a) applying onto a support a stimulable phosphor coating composition comprising a stimulable phosphor and polymer resin to form a stimulable phosphor layer, wherein the polymer resin comprises a polymer having a glass transition point of not more than 5°C. and not less than -30°C. and the polymer accounts for at least 50 weight % of the polymer resin in the stimulable phosphor layer;

(b) drying the stimulable phosphor layer; and

(c) subjecting the stimulable phosphor layer on the support to a compression treatment employing a calender roller which comes into contact with the stimulable phosphor layer to form the radiation image conversion panel, wherein the temperature of the calender roller is not less than the glass transition point of the polymer resin and not more than a glass transition point of the support and wherein the calender roller in the step (c) has a center-line mean surface roughness Ra of 0.05 to 3  $\mu\text{m}$ .